

# UNITED STATES PATENT OFFICE.

CHARLES VAN AMBURGH, OF TACOMA, WASHINGTON.

## ALLOY.

1,300,058.

Specification of Letters Patent.

Patented Apr. 8, 1919.

No Drawing.

Application filed October 2, 1917. Serial No. 194,310.

To all whom it may concern:

Be it known that I, CHARLES VAN AMBURGH, a citizen of the United States of America, residing at Tacoma, in the county 5 of Pierce and State of Washington, have invented certain new and useful Improvements in Alloys, of which the following is a specification.

This invention relates to certain new and 10 useful improvements in alloy.

The primary object of the invention is the provision of a metallic alloy and the process of making the same whereby there is provided a metal possessing a minimum coefficient of shrinkage and expansion. Such an 15 alloy is especially serviceable in connection with devices having relatively movable parts subjected to excessive heat such as the pistons of explosive motors and engines.

20 A further object of the invention is the provision of a metal presenting excessive strength but at the same time being light in weight thereby especially adapting such metal for use in manufacturing aeroplane 25 and other motors, the crank cases, cylinder blocks, and pistons being readily formed of this new alloy.

A still further object of the invention is the provision of an alloy that can be readily 30 worked for forming desired objects and can be molded with a smooth finish, the alloy having great resistance and strength as well as ductility and lightness.

My alloy consists of the following component parts:—aluminum bronze 16%, copper 1%, silicon copper 3% and pure aluminum 80%.

The aluminum bronze herein designated is 35 formed of copper 8.6%, aluminum 89% and tin 2.4% while the silicon copper is formed of 90% copper and 10% silicon.

In the process of manufacture, the aluminum bronze and silicon copper are separately formed by melting *en masse* the 45 respective elements thereof. The 16% of aluminum bronze and the 1% of copper are then melted together and when in a molten state, the 3% of silicon copper is added to the batch which becomes melted thereby and 50 enters into the constituency of the product.

The 80% of pure aluminum is then provided in ingot form and is added to the batch which is in a molten state within a suitable crucible, such addition of the aluminum 55 taking place by suspending the ingot

over the crucible and allowing the aluminum to melt in suspension while maintaining the even temperature of the batch sufficiently high to hold all of the metal in a molten state, the batch being stirred or agitated during the addition of the aluminum. This completes the forming of the alloy and may be cooled ingot or any other convenient form for use.

The percentages of the metal ingredients 60 herein noted have been found satisfactory in tests for fulfilling the objects of my invention but the same are submitted by way of example of the preferred embodiment of the formulæ for the alloy. It will be understood, however, that slightly different percentages may be used without departing from the spirit and scope of my invention as claimed.

What I claim as new is:—

1. An alloy consisting of a predominating proportion of aluminum, with substantial but smaller proportions of copper, tin and silicon.

2. An alloy consisting of substantially 80 94% of aluminum and substantial but smaller proportions of copper, tin and silicon.

3. An alloy consisting of substantially 85 94% of aluminum and 5% of copper, and equal proportions of tin and silicon.

4. An alloy consisting of substantially 80 94% aluminum, 5% copper, .38% tin and .30% silicon.

5. A process for forming an alloy consisting of melting together aluminum bronze 90 and copper, adding silicon copper and melting the same in the batch and adding aluminum.

6. The process of making an alloy consisting in first melting aluminum bronze and 95 copper, adding and melting silicon copper therein and adding pure aluminum by melting aluminum in suspension over the batch and stirring the molten batch during the addition of aluminum.

7. A process for forming an alloy consisting in melting copper, aluminum and tin and when in a molten state adding copper and silicon copper thereto and adding pure aluminum to the molten mass by suspending 105 aluminum and melting the same above the mass while maintaining the temperature of the batch sufficiently high for maintaining the metal in a molten state and stirring the batch during the adding of the aluminum.

75

80

85

90

95

100

105

110

8. A process of making an alloy consisting in forming aluminum bronze by melting together 8.6% of copper, 89% aluminum and 2.4% of tin; melting for the batch 1% of copper with 16% of the said aluminum bronze; forming silicon copper of copper

90% and silicon 10%; adding 3% of said silicon copper to the molten batch and adding 80% of pure aluminum to complete the batch.

10

In testimony whereof I affix my signature.  
CHARLES VAN AMBURGH.